

Patented Apr. 18, 1944

2,346,970

# UNITED STATES PATENT OFFICE

2,346,970

## BITUMEN AND INK MADE THEREFROM

Wilbur L. Jones, New York, N. Y., assignor to  
Interchemical Corporation, New York, N. Y., a  
corporation of Ohio

No Drawing. Application May 24, 1941,  
Serial No. 395,058

6 Claims. (Cl. 106—31)

This invention relates to asphaltic intaglio inks such as are used for printing the typical "gravure" sections of the Sunday newspapers, and is directed particularly to such an ink containing a fluxed petroleum pitch obtained from Venezuela petroleum, and to the fluxed bitumen per se.

Conventionally, inks for printing Sunday rotogravure supplements are made by dissolving gilsonite (or some other bitumen of the same type) in a volatile solvent; these are printed by intaglio process at high speeds. In order to get the desired press speeds, the inks are made with very volatile solvents (approximating the volatility of benzene) and are printed from presses equipped with closed fountains. Because of the toxicity of benzene, it has been necessary to use volatile petroleum naphthas as the principal solvent of the ink; since these do not dissolve gilsonite, it is generally necessary to use small percentages of other solvents with them. A typical satisfactory solvent formula is disclosed in the Mock Patent No. 2,139,242, issued December 6, 1938, and comprises 85-95% naphtha and 5-15% methyl ethyl ketone. Acetone, ethyl acetate and similar strong solvents may be used.

Many products which would make acceptable substitutes for gilsonite, when used with benzene as the solvent, are completely unsatisfactory when used in the petroleum naphtha active solvent mixtures which must be used. Some are insoluble; others are soluble, but dry without gloss, indicating precipitation during drying; and others retain the solvent tenaciously, and do not dry because of their poor solvent release.

A bitumen which has been suggested as a replacement for gilsonite is a petroleum pitch known as "Aruba" bitumen. It is obtained as a still bottom in the high temperature distillation of Venezuela petroleums, in the refineries at Aruba, N. W. I. It has the following approximate composition:

|                                    | Per cent   |
|------------------------------------|------------|
| Water                              | 5 to 8     |
| Volatile matter (dry basis)        | 74.24      |
| Fixed carbon                       | 25.35      |
| Ash                                | 0.41       |
| Sulfur                             | 4.80       |
| Soluble in CS <sub>2</sub> percent | 99.70      |
| Soluble in Solvesso #2 do          | 99.80      |
| Specific gravity at 60° F.         | 1.117      |
| Flash point °F.                    | 600 to 635 |

This bitumen dissolves in benzene to give a satisfactory gravure ink, of considerably higher color value than a similar ink made from gilsonite. However, the bitumen cannot be used in gravure inks, because it is insoluble in the mixtures of petroleum and active solvents used in present day gravure inks.

I have discovered that "Aruba" bitumen can be converted into a satisfactory base for gravure inks by fluxing 75 or less parts by weight of the bitumen with about one-fourth of its weight of 5 a fatty acid pitch (such as the various stearin pitches, rosin pitch, and particularly tall oil pitch) in combination with 5 or more parts by weight of a natural asphalt of the gilsonite-grahamite family.

10 If substantially less than one-quarter part of fatty acid pitch is used per part of "Aruba" bitumen (e. g.—one fifth), the fluxed product obtained is insoluble in the desired solvent mixtures; if substantially more is used (e. g.—one third), the product obtained is too soft, and dries too slowly because of solvent retention. If the fluxed mixture of bitumens contains over 75% of "Aruba," inks made therefrom yield prints with insufficient gloss; it is therefore necessary to include at least 5% of a natural bitumen of the gilsonite-grahamite family in the final product, to get enough gloss without substantially departing from the necessary "Aruba" fatty acid pitch ratio.

20 In general, I prefer to keep the added gilsonite to a minimum, since the use of more gilsonite decreases the improvement in color strength obtained by the use of the fluxed mixture, and increases the cost.

25 The mixture can be made by merely melting the three ingredients together, keeping the temperature as low as possible. Low temperature fluxing is most advantageously obtained by melting the flux, and then adding the "Aruba" and gilsonite; by this method, a temperature of 200° C. need not be exceeded.

Typical fluxed mixtures are:

### EXAMPLE 1

#### Fluxed bitumen

|                | Per cent |
|----------------|----------|
| Tall oil pitch | 18       |
| Gilsonite      | 9        |
| Aruba bitumen  | 73       |

are melted together, in order given, at 200° C. The fluxed mass has a melting point of 185° C.

50 This can be made into an ink by dissolving—

|                                                                                                | Parts by weight |
|------------------------------------------------------------------------------------------------|-----------------|
| Fluxed bitumen                                                                                 | 35              |
| Methyl ethyl ketone                                                                            | 13              |
| Lactol spirits (low solvency petroleum naphtha—evaporation rate approximating that of benzene) | 52              |

55 The ink is ready to run; its gloss and drying speed are very good, and it is considerably stronger in tone than the same ink made with gilsonite.

## EXAMPLE 2

|                 | Per cent |
|-----------------|----------|
| Tall oil pitch  | 18       |
| Cuban grahamite | 10       |
| Aruba bitumen   | 72       |

is made as in Example 1. The fluxed pitch has a melting point of 193° C. It is made into an ink as in Example 1.

## EXAMPLE 3

|                 | Per cent |
|-----------------|----------|
| Stearin pitch   | 18       |
| Cuban grahamite | 10       |
| Aruba bitumen   | 72       |

This yields an ink, when made up as in Example 1, which is superior to an ink made with gilsonite, but not quite as satisfactory as the inks of Examples 1 and 2.

Examples can of course be multiplied indefinitely without departing from the scope of my invention, which is defined in the claims. In particular, various fatty acid pitches can be used to replace those shown, although tall oil pitch is preferred. The known natural bitumens of the gilsonite-grahamite class can be used.

In making the inks, the solvents may be varied. In the preferred use of my new bitumen compositions, they are dissolved in solvent mixtures consisting predominantly of petroleum hydrocarbons having the volatility of benzene, and a minor proportion (from 5 to about 30%) of an active ketone or ester having a similar volatility (methyl ethyl ketone, acetone, methyl ethyl and isopropyl acetates, etc.). Pigments may be used with these inks, as desired. Furthermore, the fluxed bitumens disclosed may be used in other compositions to replace gilsonite (e. g., typographic inks, paints) with good success.

I claim:

1. A bitumen particularly useful as a substitute for gilsonite in intaglio printing inks, consisting essentially of a major portion of a

mixture of about 4 parts by weight of "Aruba" bitumen and 1 part by weight of fatty acid pitch, and a minor portion, comprising at least 5% by weight of the composition, of a natural asphalt of the gilsonite-grahamite group, the "Aruba" not exceeding 75% by weight of the composition.

2. A bitumen particularly useful as a substitute for gilsonite in intaglio printing inks, consisting essentially of a major portion of a mixture of about 4 parts by weight of "Aruba" bitumen and 1 part by weight of tall oil pitch, and a minor portion, comprising at least 5% by weight of the composition, of a natural asphalt of the gilsonite-grahamite group, the "Aruba" not exceeding 75% by weight of the composition.

3. A bitumen consisting of a fluxed mixture of about 72 parts by weight of "Aruba" bitumen, 18 parts tall oil pitch, and 10 parts of a natural bitumen of the gilsonite-grahamite group.

20 4. An intaglio ink comprising a solution of the bitumen of claim 1 in a solvent consisting predominantly of a petroleum hydrocarbon mixture having an evaporation rate approximating that of benzene, and a minor proportion of an oxygenated solvent of the class consisting of ketones and esters having similar volatility.

5. An intaglio ink comprising a solution of the bitumen of claim 2 in a solvent consisting predominantly of a petroleum hydrocarbon mixture having an evaporation rate approximating that of benzene, and a minor proportion of an oxygenated solvent of the class consisting of ketones and esters having similar volatility.

30 6. An intaglio ink comprising a solution of the bitumen of claim 3 in a solvent consisting predominantly of a petroleum hydrocarbon mixture having an evaporation rate approximating that of benzene, and a minor proportion of an oxygenated solvent of the class consisting of ketones and esters having similar volatility.

40

WILBUR L. JONES.